

Nov. 4, 1969

E. GLAESENER

3,476,549

PROCESS FOR CASTING OF METAL FROM A REFINING  
FURNACE INTO A LADLE

Filed Nov. 28, 1966



ERNEST GLAESENER  
INVENTOR.

BY

*Karl G. Ross*  
Attorney

1

3,476,549

**PROCESS FOR CASTING OF METAL FROM A  
REFINING FURNACE INTO A LADLE**  
Ernest Glaesener, Dudelange, Luxembourg, assignor to  
ARBED, Acieries Reunies de Burbach-Eich-Dudelange,  
S.A., Luxembourg, Luxembourg, a corporation of  
Luxembourg

Filed Nov. 28, 1966, Ser. No. 597,462  
Claims priority, application Luxembourg, Dec. 7, 1965,  
50,017  
Int. Cl. C22c 33/00; B22d 11/10  
U.S. Cl. 75—46

1 Claim

## ABSTRACT OF THE DISCLOSURE

A method of casting steel from a refining furnace into a ladle for the transportation of the steel in which a tube is connected to the refining furnace at air air-tight junction and leads the molten steel from a point in the furnace below its slag layer to the ladle close to its bottom and beneath the slag layer therein. Deoxidation and alloying materials are introduced into the steel through another tube leading below the slag layer in the ladle.

The present invention relates to a process for casting metal, especially steel, from a refining furnace into a ladle, and is characterised by the feature, that any contact of the cast-metal jet with the surrounding air is prevented.

It is well known that the main object of the steel-refining process lies in obtaining a metal or alloy having a definite chemical composition. It is therefore quite important, that during casting of refined metal or steel no change in the chemical composition of such metal or alloy may occur, and that no contact of the metal with the oxygen of air should take place. The same is true for slag, as particles of slag can be carried along with metal when cast. A change in the composition of slag means a disturbance of the equilibrium existing between refined metal and slag and brings about a change in the composition of metal as well.

According to the present invention no contact of the cast metal with the oxygen of air takes place and particles of slag can reach the bottom of the cast metal column, and can then easily and rapidly rise to the surface of the metal bath and facilitate decantation, since there exists a considerable difference between the density of metal and that of slag.

The present invention therefore concerns a process for casting metal with the object, that practically no change of the composition of the refined metal will take place during casting of such metal from the refining furnace into the ladle.

According to the present invention any access of air to the jet of cast metal is avoided by casting from the refining furnace takes place through a tube fixed to the tap hole of the refining furnace and reaching nearly to the bottom of the ladle used. In this manner, oxydation of the metal jet during the casting operation is completely made impossible. Maintenance of the metal composition, as it has been realised at the end of the refining operation, is therefore guaranteed during casting into the ladle. No change of composition due to slag carried along with the cast metal can occur, since the movement of such slag particles through liquid metal takes place solely in the absence of air. According to the present invention any disturbance of the equilibrium prevailing at the end of the refining operation is therefore carefully avoided.

According to the present invention there is no formation during casting of non-metallic inclusions, as will occur with known processes due to oxydation by air of the metal jet and due to slag particles remaining in the metal

2

bath and not rising to the surface layer of slag. According to the present invention the slag particles will first penetrate deep into the metal bath and will then rapidly rise to the surface of the bath, as their lower density much differs from the density of the molten metal. This is of great practical importance, since according to the invention no contamination of the refined metal can happen.

According to the present invention the addition of alloying and deoxydation agents also is carried out with a tube reaching to a certain depth into the metal bath and below its surface layer of slag. This procedure is of great practical advantage, as such additives are often introduced into the ladle containing or being filled with refined metal, as for example liquid ferro-manganese. In this manner no oxydation or other undesired reaction with air of these additives is permitted. The added agents will immediately and without alteration get in contact with the metal bath to be treated. According to the invention deoxydation can proceed more easily and alloying agents can directly act in their original state without being oxidized or otherwise altered with a risk of contamination for the refined metal. No reaction of these additives with the slag can take place, since the tube used for their introduction will reach beneath the surface layer of slag. As a result a better yield of alloy is made possible.

It is further very advantageous according to the present invention to add to the liquid metal relatively light alloying and deoxydation agents, as for example aluminum. According to known practice, additives with lower density will not always penetrate deeply enough into the metal bath and cannot therefore spread uniformly to give a homogeneous product.

Another important advantage offered by the present invention is the fact that, when phosphoric anhydride is present in the slag, rephosphorization can practically be completely avoided, since there is no disturbance of the existing equilibrium.

The accompanying sole figure of the drawing is a schematic arrangement of a device to be used according to the present invention, in cross-section with the aid of the drawing the following example is given in order to better illustrate the invention.

The metal leaving the refining furnace 1 through tap hole 2 flows through casting tube 3 into the ladle 4 being placed on the transport car 5. The lower part of the casting tube 3 almost reaches the bottom of the ladle and will therefore quickly be immersed into the liquid-metal bath 7. As soon as the surface of the bath in the ladle has reached a certain height, the tube 6 used for the introduction of alloying and deoxydation agents is plunged through the layer of slag 8 into the metal bath. If relatively heavy agents are to be added, as for example ferro-manganese in pieces, addition will be directly carried out through the tube used as such. In the case of additives with a lower density however, the tube used for their introduction is first closed at its lower end by means of a thin sheet and after having received the additives is plunged to a greater depth into the metal bath and immediately afterwards is slightly drawn back in order to leave the additives at such depth, after the sheet has been melted. When proceeding in this manner, attention is to be paid to make sure that the tube remains immersed beneath the surface layer of slag.

The tube 3 used according to the invention can be made of a refractory material or of metal. As a metal or metal alloy use can be made either of one being resistant to the bath at the temperature of the fluid metal bath or of one being melted at such temperature. In the latter case the metal has to be chosen in such a manner as to always keep the lower end of the tube beneath the surface of the metal bath in the ladle.

What is claimed is:

1. A method of casting molten steel from a refining furnace containing a bath of the molten steel covered by a slag layer into a casting ladle for transportation away from said refining furnace, comprising the steps of affixing a downwardly extending air-tight tube of refractory material in an air-tight manner in registry with a tap hole formed in said furnace below the surface of the bath of molten steel therein and below the slag layer above said bath, and positioning said tube and said ladle such that said tube opens into said ladle close to the bottom of the ladle and is trained on the bottom thereof; draining molten steel from said furnace through said tube into said ladle with entrainment of some slag to form a rising bath of molten steel in said ladle surmounted by a slag layer accumulated from slag entrained with the molten steel passing through said tube; and then completing the tapping of the molten steel from said furnace into said ladle

through said tube beneath the slag layer on the bath previously introduced into said ladle.

#### References Cited

##### UNITED STATES PATENTS

- 5 2,577,764 12/1951 Hulme *REMOVING MOLTEN METAL FROM FURNACE*  
2,803,861 8/1957 Prucha et al. *REMOVING MOLTEN METAL* 164—337  
2,976,587 3/1961 Daussan *REMOVING MOLTEN METAL* 164—133 X

##### FOREIGN PATENTS

- 10 228,418 1963 Austria.

L. DEWAYNE RUTLEDGE, Primary Examiner

G. K. WHITE, Assistant Examiner

U.S. CL. X.R.

15 75—61; 266—38